# EUROPEAN PATENT SPECIFICATION

(11) **EP 2 867 393 B1**
(45) Date of publication and mention of the grant of the patent: **02.12.2020**
(21) Application number: 13889765.7
(22) Date of filing: 09.09.2013
(51) Int. Cl.: D02G 3/32, D02G 3/36, D02G 3/38

(54) **CORE SPUN ELASTIC COMPOSITE YARN AND WOVEN FABRIC THEREOF**
ELASTISCHES VERBUNDKERNGARN UND GEWEBE DARAUS
FIL COMPOSITE ÉLASTIQUE FILÉ À ÂME ET TISSU TISSÉ LE COMPRENANT

(43) Date of publication of application: 06.05.2015
(73) Proprietor: Texhong Textile Group Limited, Quarry Bay Hong Kong (CN)
(72) Inventor: YUNG, Wing Kay Leo, Hong Kong (CN)
(74) Representative: Modiano, Micaela Nadia
(86) International application number: PCT/CN2013/083149
(87) International publication number: WO 2015/032097

(56) References cited:
- CN-A- 101 115 874
- CN-A- 101 994 186
- GB-A- 949 326
- JP-A- H0 693 531
- US-A1- 2008 268 734

## Description

### FIELD OF THE INVENTION

The present invention relates to core spun elastic composite yarn having a fibrous sheath covering an elastic performance filament and a staple spun yarn. In particular, the present core spun yarn is woven into fabrics exhibiting excellent stretch, recovery, hand feel characteristics and improved yarn piecing properties.

### BACKGROUND

Conventional stretch fabric is commonly made up of core spun spandex yarn. Warping and/or filling of the conventional core spun spandex yarn result in fabric of high shrinkage and stretchability which requires additional finishing process, such as heat setting. Generally, the conventional stretch fabric is associated with drawbacks, such as limited elongation and growth, and stability of the fabric width are being affected.

Elastic bi-component polyester filament has been disclosed in US Pat. No. 3,671,379 and woven stretch fabrics comprising this bi-component polyester filament is disclosed in US Pat. No. 5,922,433, US Pat. No.7,143,790 and US Pat. No, 7,299,828. However, these fabrics woven from bare bi-component polyester filament have a strong synthetic feel and look. Such fabrics are therefore limited to be used in filling and denim. Moreover, piece dyeing these woven stretch fabrics of bi-component polyester filament must be performed in two separate dyeing processes and elongation of the fabric is inevitably affected.

US Pat. No. 7,310,932 discloses fabric made up of core spun yarn comprising bi-component polyester filament covered with staple fibers. Although the fabric disclosed in the '932 patent is associated with improved appearance and hand-feel, grinning effect and limited elongation of the fabric remain.

US Pat. No. US 7,299,828 B2 and US 8,093,160 disclose fabric made up of core spun yarn containing at least one elastic performance filament and at least one inelastic or elastic filament. Woven fabric made of such yarns can have a good elongation and recovery, but the existing problem of grinning effect, low piecing strength and synthetic texture remains unsolved.

As a result, there is a need to develop a new core spun composite yarn that produces fabrics with desirable stretchability, good recovery, hand feel, reduced grinning and improved piecing characteristics.

### SUMMARY OF THE INVENTION

The objective of the present invention is to provide a new core spun elastic composite yarn having excellent elongation, excellent recovery, and better hand feel properties, and to solve the problem of grinning effect and low yarn piecing strength at the piecing position as compared to existing composite yarns. The present composite yarn is suitable for denim, warp and filling. The present invention is a core spun elastic composite yarn comprising at least one elastic performance filament, and at least one staple spun yarn. The elastic performance filament ranges from about 20 denier to about 140 denier (linear density of 2.22 x 10⁻⁶ kg/m to 1.56 x 10⁻⁵ kg/m). The staple spun yarn has an English cotton yarn count (Ne) ranging from about 8 to about 100 (linear density of 7.38 x 10⁻⁵ kg/m to 5.91 x 10⁻⁶ kg/m), preferably from about 20 to 60 (linear density 2.95 x 10⁻⁵ kg/m to 9.87 x 10⁻⁶ kg/m).

A fibrous sheath of at least one staple fiber surrounds the at least one elastic performance filament and the at least one staple spun yarn. Said fibrous sheath may be staple fibers such as cotton, polyester, nylon, rayon, wool, acrylic and a combination thereof. In general, there is no restriction on the type of staple fibers that can be used in the present invention as long as the properties of the present invention are unaffected. The fibrous sheath ranges from English cotton yarn count from about Ne 4 to Ne 60 (linear density of 0.000148 kg/m to 9.87 x 10⁻⁶ kg/m). In yet another embodiment, the fibrous sheath ranges from Ne 7 to Ne 40 (linear density of 8.44 x 10⁻⁵ kg/m to 1.48 x 10⁻⁵ kg/m).

Another objective of the present invention is to provide a textile fabric woven from the core spun elastic composite yarn of the present invention. In a particular embodiment, the textile fabric is a denim fabric.

### BRIEF DESCRIPTION OF THE DRAWINGS

**FIG. 1** is a side view of a process and apparatus for manufacturing the core spun elastic composite yarn in accordance with one embodiment of the present invention.
**FIG. 2** is a front view of a process and apparatus for manufacturing the core spun elastic composite yarn in accordance with one embodiment of the present invention.
**FIG. 3** is a side view of a process and apparatus for manufacturing the core spun elastic composite yarn not in accordance with the present invention.
**FIG. 4** is a front view of the process and apparatus for manufacturing the core spun elastic composite yarn shown in Fig. 3 not in accordance with the present invention.
**FIG. 5** is a side view of a process and apparatus for manufacturing the core spun elastic composite yarn not in accordance with the present invention.
**FIG. 6** is a side view of the process and apparatus for manufacturing the core spun elastic composite yarn shown in Fig. 5 not in accordance with the present invention.
**FIGs. 7** show piecing position of elastic yarn with one elastic performance filament and one inelastic polyester filament **(****FIG. 7a****),** and piecing position of elastic yarn with one elastic performance filament and one staple spun yarn **(****FIG. 7b****).**
**FIG. 8** is a table showing the physical properties of textile fabrics woven from three exemplary embodiments of the present invention.

### DEFINITIONS

"Warp" means the lengthwise threads in a woven fabric.
"Filling" or "weft" means threads widthwise in a fabric as woven.
"Spandex" means a manufactured fiber with good elasticity in which the fiber-forming substance is a long-chain synthetic polymer comprised of at least 85% of segmented polyurethane.
"Filament" means a fibrous of indefinite length.
"Fiber" means a fibrous strand of definite length, such as staple fiber.
"Yarn" means a product of substantial length and relatively small cross-section consisting of fibers and/or filament(s) with or without twist.
"Sliver" means an assemblage of fibers in continuous form without twist.
"Roving" is a name given, individually or collectively, to the relatively fine fibrous strands used in the later or final processes of preparation for spinning.
"Spinning" means the drafting and where appropriate the insertion of twist in natural or staple man-made fibers to form a yarn.
"Core Yarn" means a yarn consisting of a number of component yarns, of which one or more are constrained to lie permanently at the central axis of the composite thread, whilst the remaining yarns act as covering yarns.
"Spun yarn" means a yarn that consists of staple fibers held together usually by twist.
"Core spun yarn" means a yarn consisting of a yarn surrounded by staples fibers. The yarn has the strength and/or elongation of the central thread whilst exhibiting most of the other characteristics of the surface staple fibers.
"Draft ratio" or "Draft" is the ratio between length of a stock filamentary strand from a package thereof which is fed into a spinning machine to the length of the filamentary strand delivered from the spinning machine. A draft ratio of greater than 1.0 is thus a measure of the reduction in bulk and weight of the stock filamentary strand.
"Elastic recovery" means the immediate change in elongation experienced by a textile during a loading cycle when, after being held at a defined elongation for a defined time, the applied tension is removed.

Definitions of the above terms and any other technical terms used herein are as readily would be understood by one skilled in the art in the field of textile and as defined in the Textile Terms and Definitions (9th Edition) by The Textile Institute, UK.

### DETAILED DESCRIPTION OF THE INVENTION

The present core spun elastic composite yarn comprises at least one elastic performance filament, at least one staple spun yarn and a fibrous sheath comprised of a mass of staple fibers. Said fibrous sheath surrounds the at least one elastic performance filament and the at least one staple spun yarn independently. In another embodiment not according to the invention, the at least one elastic performance filament and the at least one staple spun yarn are first twisted together to form a central thread and the fibrous sheath surrounds said central thread.

Any commercially available elastic performance filament may be employed in the present composite yarn. In one embodiment, the elastic performance filament is made from spandex or lastol polymers. Other elastic performance filaments include, but are not limited to, ethylene/α-olefin interpolymers. U.S. Pat. Nos. 5,272,236, 5,278,272, 5,322,728, 5,472,775, 5,645,542, 6,140,442 and 6,225,243 disclose various examples of elastic performance filaments applicable for the present invention. The elastic performance filament of the present invention typically has 4.44×10⁻⁶ kg/m - 1.56×10⁻⁵ kg/m (40 to 140 denier) and 1% to 40% of total weight of the composite yarn. In another embodiment, the draft of the elastic performance filament typically ranges from 1.5 to 5.0.

Document JPH0693531 discloses a process for producing a bulky textile structure having good feeling and clothing comfort and excellent form-stability, water and sweat- absorption and heat-insulation. The structure is a thermoplastic synthetic fiber filament yarn 2 helically wound around filament yarn 1 of a water-soluble polyvinyl alcohol or spun staple fiber yarn of a water-soluble polyvinyl alcohol to obtain covering yarn. A fiber structure formed of multilayer structure yarn produced by using the covering yarn as core yarn and a cellulosic staple fiber as the outer layer is treated in a water bath to dissolve the water-soluble polyvinyl alcohol fiber constituting the core yarn.

Document GB949326 discloses an elastic yarn comprising a low twist strand formed of a multiplicity of loosely-arranged staple length fibres, an elastomeric thread and a continuous strand of high strength if compared to the former strand. The low twist strand and the thread are so arranged that when the thread is contracted the strand is loosely associated therewith and the low twist strand, the thread and the continuous strand are arranged so that when the thread is elongated the fibres of the strand are pressed against the thread throughout the length of the strand.The low twist strand may be formed of cotton, nylon, polyester or polyacrylic fibres. The thread may be natural or synthetic rubber e.g.polyurethanes and may be either untwisted or pre-twisted. The continuous strand may be a spun yarn, a continuous mono-filament or a continuous multifilament yarn preferably of low twist e.g.five turns per inch.

The staple spun yarn of the present composite yarn may be made of any material known to those skilled in the art. Examples of staple spun yarn suitable for the present invention include, but are not limited to, natural, re-generated, synthetic, dyed and non-dyed fibers. The present staple spun yarn may be s-twist or z-twist. The staple spun yarn has an English cotton count ranges 7.38 x 10⁻⁵ kg/m - 5.91 x 10⁻⁶ kg/m (Ne 8 to Ne 100). In one embodiment, the English cotton count is 2.95 x 10⁻⁵ kg/m - 9.87 x 10⁻⁶ kg/m (Ne 20 to Ne 60). In another embodiment, the present staple spun yarn is about 4% to 50% of the total weight of the present composite yarn. In yet another embodiment, the draft of the staple spun yarn is 1.0 to 1.3.

The fibrous sheath is formed from a relatively dense mass of randomly oriented entangled spun synthetic staple fibers (e.g. polyamides, polyesters and the like) or spun natural staple fibers. Other examples include, but are not limited to, cotton, viscose rayon, polyester, wool, acrylic or a combination thereof. Particularly, the fibrous sheath may be ring-spun from a roving of staple fibers and forms an incoherent mass of entangled spun staple fibers. Length of the staple fiber is not critical. The linear density of the fibrous sheath ranges from 0.000148 kg/m - 9.87×10⁻⁶ kg/m(Ne 4 to Ne 60). In yet another embodiment, the fibrous sheath ranges from 8.44×10⁻⁵ kg/m - 1.48×10⁻⁵ kg/m(Ne 7 to Ne 40).

The present core spun elastic composite yarn may be used as a warp and/ or filling yarn to form woven fabrics exhibiting excellent recovery characteristics. The present composite yarn has a yarn count ranges 0.000148 kg/m - 9.87×10⁻⁶ kg/m(Ne 4 to Ne 60), preferably 8.44×10⁻⁵ kg/m - 1.48×10⁻⁵ kg/m(Ne 7 to Ne 40). In one embodiment, the fabric woven from the present composite yarn is a plain weave, twill weave or satin weave pattern. Such fabrics in accordance with the present invention have at least about 20% stretch or greater. More specifically, fabrics in accordance with the present invention exhibit improved less synthetic hand-feel, improved hairiness, resistant to abrasion as compared to existing composite yarns, such as those having a filament core/ central thread of an elastic filament combining with an inelastic/ elastic filament. Fabrics of the present invention also have reduced or no grinning effect and high piecing strength, thereby efficiency of the weaving process is improved. When the present composite yarn is made of 100% cotton or rayon/cotton blend, the common white spot problem occurring in denim fabric is eliminated when the composite yarn is used as warp. Furthermore, 100% cotton or rayon/cotton blend of the present composite yarn also avoids two dyeing processes for piece dyed fabrics.

The present composite yarn may be manufactured by any staple fiber spinning process, such as core spinning, ring spinning and the like as readily known by those skilled in the art. Process and apparatus for making the present elastic core spun composite yarn is shown in **FIGs. 1** and **2****.** During the spinning process, the elastic performance filament **21** and staple spun yarn **22** are unwound from the tube **34** & **35** respectively in the direction of **41 & 42** at different speed according to the desired draft. The draft of elastic performance filament is calculated by the ratio of the surface speed of front roller **31** and the tube **34,** whereas the draft of staple spun yarn is calculated by the ratio of the surface speed of front roller **31** and the tube **35.** In one embodiment of the present invention, the elastic performance filament has a draft which is at least twice or three times the draft of the staple spun yarn.

The staple fibers or roving **13** and **14** are unwound from tube **11** and **12** to meet the elastic performance filament **21** and staple spun yarn **22** at the front roller **31.** The position of the elastic performance filament on the roving **13** is adjusted by roller **36** and guide **38** whereas the position of staple spun yarn **22** on the roving **14** is adjusted by roller **37** and guide **39.** As depicted in **FIG. 2****,** elastic performance filament **21** and staple spun yarn **22** are individually twisted with staple fibers or roving **13** and **14** first, and thereafter twisted together at the front roller **31** forming the present core spun elastic composite yarn. The alignment of the elastic performance filament **21** and staple spun yarn **22** on the roving can effectively reduce the grinning effect. The present core staple spun yarn has reduced grinning effect and improved piecing strength at the piecing position.

Another embodiment not according to the present invention of process and core spinning apparatus to make a composite yarn is shown in **FIGs. 3** and **4****.** The elastic performance filament **21** and that staple spun yarn **22** are unwound from the tubes **34** and **35** respectively in the directions of **41** and **42** at different speed according to the desired draft. Filament **21** and yarn **22** are twisted together by roller **36** first forming a filament strand/ central thread, thereafter staple fibers or roving **of 13** and **14** are twisted around the filament strand to form core spun yarn **1**. The position of the elastic performance filament **21** and staple spun yarn **22** on the staple fibers or roving **13** and **14** is adjusted by roller **36** and guides **38** and **39.**

Another embodiment not according to the present invention of a core spinning apparatus is shown in **FIGs. 5** and **6****,** wherein the elastic performance filament is twisted with the staple spun yarn to form a central strand **23** beforehand. The apparatus that is useful in twisting the elastic performance filament with the staple spun yarn includes, but is not limited to, a ring spinning machine, an open end spinning machine and a vortex spinning machine. The filamentary strand is unwound from the tube **34** in the direction **41.** The draft of central strand is calculated by the ratio of the surface speed of front roller **31** and the tube **34.** The staple fibers or roving **13** and **14** are unwound from the tubes **11** and **12** to meet central strand **23** at the front roller **31.** The position of the core staple spun yarn on the roving **13** and **14** is adjusted by roller **36** and guides **38** and **39.**

The grinning effect of the conventional elastic core yarn which comprises an elastic performance filament and inelastic or elastic filament at the piecing position is shown in **FIG. 7a****.** The present invention of elastic core spun composite yarn comprising elastic performance filament and staple spun yarn as the filament core has no grinning effect at the piecing position **(****FIG. 7b**). The present elastic core spun composite yarn can be used to provide a woven stretch fabric designed as a filling stretch, warp stretch or bi-stretched by using the elastic core spun composite yarn in a warp, weft or filling and warp directions respectively. Stretch fabric woven from the present composite yarn may have a fabric weight ranging from 135.623 g/m² - 542.492 g/m²(4 oz/square.yard to 16 oz/square.yard (oz/sq.yd)).

The following are textile fabrics woven from exemplary embodiments of the present invention and the associated properties **(****FIG. 8****).**

### Example 1: Denim Weft Stretch Fabric

A denim stretch fabric having a weft yarn 3.69×10⁻⁵ kg/m(Ne 16) in accordance with the present invention. The weft yarn includes cotton fibrous sheath and a core polyester staple spun yarn 1.31×10⁻⁵ kg/m(Ne 45) and spandex of 4.44×10⁻⁶ kg/m(40 denier). The denim stretch fabric exhibits good elongation (27.4%) and growth (3.0%).

### Example 2: Denim Weft Stretch Fabric

The weft yarn of 3.69×10⁻⁵ kg/m(Ne 16) in accordance with the present invention comprises a core strand of 100% cotton spun yarn 1.31×10⁻⁵ kg/m(Ne 45) and spandex of 4.44×10⁻⁶ kg/m(40 denier) covered by 100% cotton fibrous sheath. The fabric has good elongation (34.6%) and growth (5.4%). The fabric exhibits 100% cotton feel and no grinning effect in the fabric and at the piecing position. The present core strand of Example 2 is also useful as warp.

### Example 3: Denim Weft Stretch Fabric

The weft with 100% cotton fibrous sheath and a core polyester staple spun yarn 9.87×10⁻⁶ kg/m(Ne 60) and spandex of 4.44×10⁻⁶ kg/m(40 denier). Good elongation (30.1%) and growth (3.6%) are exhibited in the fabric woven therefrom.

## Claims

1. A core spun elastic [] composite yarn (1) comprising: at least one elastic performance filament (21) and at least one staple spun yarn (22), and a fibrous sheath of at least one staple fiber (13, 14) that surrounds the at least one elastic performance filament and the at least one staple spun yarn, wherein the elastic performance filament has a linear density of 2.22x10⁻⁶kg/m to 1.56 x 10⁻⁵kg/m (denier from 20 to 140), the staple spun yarn has a linear density of 7.38x10⁻⁵kg/m to 5.91 x 10⁻⁶kg/m (English cotton yarn count (Ne) from 8 to 100) and said fibrous sheath of at least one staple fiber has a linear density of 0.000148kg/m to 9.87 x 10⁻⁶kg/m (English cotton yarn count (Ne) from 4 to 60), wherein said at least one elastic performance filament and said at least one staple spun yarn individually twist with said fibrous sheath, and said at least one elastic performance filament surrounded with fibrous sheath and said at least one staple spun yarn surrounded with fibrous sheath twist together forming the composite yarn.

2. The composite yarn of claim 1, wherein the staple spun yarn (22) has a linear density of 2.95x10⁻⁵kg/m to 9.87 x 10⁻⁶kg/m (English cotton yarn count (Ne) from 20 to 60).

3. The composite yarn of claim 1, wherein said fibrous sheath of at least one staple fiber (13, 14) has a linear density of 8.44x10⁻⁵kg/m to 1.48 x 10⁻⁵kg/m (English cotton yarn count (Ne) from 7 to 40).

4. The composite yarn of claim 1, wherein the elastic performance filament (21) is 1 percent to 40 percent of total weight of the composite yarn and the staple spun yarn (22) is 4 percent to 50 percent of total weight of composite yarn.

5. The composite yarn of claim 1, wherein said fibrous sheath comprises natural or synthetic staple fibers or a combination thereof.

6. The composite yarn of claim 1, wherein said at least one staple spun yarn is made of natural staple fibers, re-generated staple fibers, synthetic staple fibers or a combination thereof.

7. The composite yarn of claim 1, wherein the draft of the elastic performance filament is from 1.5 to 5.0.

8. A woven stretch fabric comprising the composite yarn of claim 1 as warp or filling yarn or both.

9. The woven stretch fabric in claim 8, wherein the fabric is a plain woven, twill, satin, or denim.

10. The woven stretch fabric in claim 8, wherein the fabric is denim.

11. The woven stretch fabric in claim 8, wherein warp or filling or both have an elongation from 10% to 40%.

## Patentansprüche

1. Ein elastisches Verbundkerngarn (1), das Folgendes umfasst:
mindestens ein elastisches Leistungsfilament (21) und mindestens ein Stapel-Spinnfasergarn (22) und eine faserige Hülle mindestens einer Stapelfaser (13, 14), die das mindestens eine elastische Leistungsfilament und das mindestens eine Stapel-Spinnfasergarn umgibt, wobei das elastische Leistungsfilament eine Lineardichte von 2,22 x 10⁻⁶ kg/m bis 1,56 x 10⁻⁵ kg/m (Denier von 10 bis 140) hat, das Stapel-Spinnfasergarn eine Lineardichte von 7,38 x 10⁻⁵ kg/m bis 5,91 x 10⁻⁶ kg/m (Englische Garnnummer (Ne) von 8 bis 100) hat und die faserige Hülle mindestens einer Stapelfaser eine Lineardichte von 0,000148 kg/m bis 9,87 x 10⁻⁶ kg/m (Englische Garnnummer (Ne) von 4 bis 60) hat, wobei das mindestens eine elastische Leistungsfilament und das mindestens eine Stapel-Spinnfasergarn sich einzeln mit der faserigen Hülle verdrillen und das mindestens eine elastische Leistungsfilament, dass mit der faserigen Hülle umgeben ist und das mindestens eine Stapel-Spinnfasergarn, dass mit faseriger Hülle umgeben ist sich miteinander verdrillen um das Verbundgarn zu bilden.

2. Das Verbundgarn gemäß Anspruch 1, wobei das Stapel-Spinnfasergarn (22) eine Lineardichte von 2,95 x 10⁻⁵ kg/m bis 9,87 x 10⁻⁶ kg/m (Englische Garnnummer (Ne) von 20 bis 60) hat.

3. Das Verbundgarn gemäß Anspruch 1, wobei die faserige Hülle mindestens einer Stapelfaser (13, 14) eine Lineardichte von 8,44 x 10⁻⁵ kg/m bis 1,48 x 10⁻⁵ kg/m (Englische Garnnummer (Ne) von 7 bis 40) hat.

4. Das Verbundgarn gemäß Anspruch 1, wobei das elastische Leistungsfilament (21) 1 Prozent bis 40 Prozent des Gesamtgewichts des Verbundgarns ausmacht und das Stapel-Spinnfasergarn (22) 4 Prozent bis 50 Prozent des Gesamtgewichts des Verbundgarns ausmacht.

5. Das Verbundgarn gemäß Anspruch 1, wobei die faserige Hülle natürliche oder synthetische Stapelfasern oder eine Kombination davon umfasst.

6. Das Verbundgarn gemäß Anspruch 1, wobei das mindestens eine Stapel-Spinnfasergarn aus natürlichen Stapelfasern, Regenerat-Stapelfasern, synthetischen Stapelfasern oder einer Kombination davon besteht.

7. Das Verbundgarn gemäß Anspruch 1, wobei der Verzug des elastischen Leistungsfilament von 1,5 bis 5,0 beträgt.

8. Ein Stretchgewebe dass das Verbundgarn gemäß Anspruch 1 als Kettfaden oder Schussfaden oder beides umfasst.

9. Das Stretchgewebe in Anspruch 8, wobei das Gewebe eine einfache Webware Twill, Satin oder Denim ist.

10. Das Stretchgewebe in Anspruch 8, wobei das Gewebe Denim ist.

11. Das Stretchgewebe in Anspruch 8, wobei der Kett- oder Schussfaden oder beide eine Bruchdehnung von 10% bis 40% haben.

## Revendications

1. Fil composite élastique filé à âme (1) comprenant : au moins un filament à performance élastique (21) et au moins un fil filé à fibres discontinues (22) et une gaine fibreuse d'au moins une fibre discontinue (13, 14) qui entoure le au moins un filament à performance élastique et le au moins un fil filé à fibres discontinues, dans lequel le filament à performance élastique a une densité linéaire de 2,22 x 10⁻⁶ kg/m à 1,56 x 10⁻⁵ kg/m (denier de 20 à 140), le fil filé à fibres discontinues a une densité linéaire de 7,38 x 10⁻⁵ kg/m à 5,91 x 10⁻⁶ kg/m (numéro de fil de coton anglais (Ne) de 8 à 100) et ladite gaine fibreuse d'au moins une fibre discontinue a une densité linéaire de 0,000148 kg/m à 9,87 x 10⁻⁶ (numéro de fil de coton anglais (Ne) de 4 à 60), dans lequel ledit au moins un filament à performance élastique et ledit au moins un fil filé à fibres discontinues se torsadent individuellement avec ladite gaine fibreuse et ledit au moins un filament à performance élastique s'est entouré de la gaine fibreuse et ledit au moins un fil filé à fibres discontinues s'est entouré de la torsade à gaine fibreuse, ensemble, formant le fil composite.

2. Fil composite selon la revendication 1, dans lequel le fil filé à fibres discontinues (22) a une densité linéaire de 2,95 x 10⁻⁵ kg/m à 9,87 x 10⁻⁶ kg/m (numéro de fil de coton anglais (Ne) de 20 à 60).

3. Fil composite selon la revendication 1, dans lequel ladite gaine fibreuse d'au moins une fibre discontinue (13, 14) a une densité linéaire de 8,44 x 10⁻⁵ kg/m à 1,48 x 10⁻⁵ kg/m (numéro de fil de coton anglais (Ne) de 7 à 40).

4. Fil composite selon la revendication 1, dans lequel le filament à performance élastique (21) fait 1 pour cent à 40 pour cent du poids total du fil composite et le fil filé à fibres discontinues (22) fait 4 pour cent à 50 pour cent du poids total du fil composite.

5. Fil composite selon la revendication 1, dans lequel ladite gaine fibreuse comprend des fibres discontinues naturelles ou synthétiques ou une combinaison de celles-ci.

6. Fil composite selon la revendication 1, dans lequel ledit au moins un fil filé à fibres discontinues est fait de fibres discontinues naturelles, de fibres discontinues régénérées, de fibres discontinues synthétiques ou d'une combinaison de celles-ci.

7. Fil composite selon la revendication 1, dans lequel l'étirage du filament à performance élastique va de 1,5 à 5,0.

8. Tissu extensible tissé, comprenant le fil composite selon la revendication 1 en tant que fil de chaîne ou fil de trame ou les deux.

9. Tissu extensible tissé selon la revendication 8, dans lequel le tissu est à armure toile, un croisé, un satin ou un denim.

10. Tissu extensible tissé selon la revendication 8, dans lequel le tissu est du denim.

11. Tissu extensible tissé selon la revendication 8, dans lequel la chaîne ou la trame ou les deux ont une extensibilité de 10 % à 40 %.
